

# UNITED STATES PATENT OFFICE.

JOSEPH M. FLANNERY, OF PITTSBURGH, PENNSYLVANIA, ASSIGNOR TO STANDARD CHEMICAL COMPANY, OF PITTSBURGH, PENNSYLVANIA.

## IRON ALLOY.

1,247,252.

Specification of Letters Patent. Patented Nov. 20, 1917.

No Drawing.

Application filed February 19, 1916. Serial No. 79,432.

*To all whom it may concern:*

Be it known that I, JOSEPH M. FLANNERY, a citizen of the United States, and a resident of Pittsburgh, in the county of Allegheny and State of Pennsylvania, have invented certain new and useful Improvements in Iron Alloys; and I do hereby declare the following to be a full, clear, and exact description of the invention, such as will enable others skilled in the art to which it appertains to make and use the same.

This invention relates to iron alloys, one object of the invention being to alloy another metal with cast iron or with semi-steel, which will increase the strength and toughness of the iron; increase the fluidity of the same; enhance the quality of the iron to facilitate the machining of the same; to increase the resistance of the iron to wear; improve the molecular structure, and increase the quality of shrinkage in the molding process.

With these and other objects in view, the invention consists in an iron alloy, as hereinafter described and pointed out in the claim.

My improved alloy comprises cast iron or semi-steel having uranium alloyed therewith in the proportion approximately from .05% to 1% uranium. The uranium may be supplied to the molten iron either in the form of uranium metal or ferro-uranium in such quantity as will result in a uranium

content in the finished product of from .05% to 1% as above stated. The uranium metal or ferro-uranium should be added to the stream of molten iron as it passes from the cupola into the ladle; or a small quantity of molten iron may be poured into a crucible, to which the uranium metal or ferro-uranium may be added, and this may be followed by the pouring of the balance of the metal.

The uranium when alloyed with cast iron or semi-steel acts as a de-oxidizing and de-nitrogenizing agent, increases the tensile strength of the iron and its resistance to wear and produces a finer grain casting. It also gives to the iron a quality which will increase its fluidity when in a molten state, and also facilitate shrinkage when being molded, and imparts to the iron a quality which will facilitate the machining thereof.

Having fully described my invention what I claim as new and desire to secure by Letters-Patent, is:

An iron or semi-steel alloy consisting of cast iron or semi-steel having from .05% to 1% of uranium alloyed therewith.

In testimony whereof, I have signed this specification in the presence of two subscribing witnesses.

JOSEPH M. FLANNERY.

Witnesses:

WILLIAM GANLEY,  
H. B. KEOWEY.